

1

3,843,318

**PROCESS FOR DYEING CELLULOSE FIBRES**

Hans-Ulrich von der Eltz, Frankfurt am Main, Germany,  
assignor to Farbwerke Hoechst Aktiengesellschaft  
vormals Meister Lucius & Bruning, Frankfurt am Main,  
Germany

No Drawing. Continuation of abandoned application Ser. No. 706,766, Feb. 20, 1968. This application Oct. 12, 1970, Ser. No. 80,155

Claims priority, application Germany, Feb. 28, 1967, F 51,665; Apr. 12, 1967, F 52,106  
Int. Cl. D06p 1/02, 1/24, 1/68

U.S. CL. 8—1 L

5 Claims

### ABSTRACT OF THE DISCLOSURE

Process for pad-dyeing textile materials made of native or regenerated cellulose fibres with reactive dyestuffs having as a group capable of reacting with the hydroxyl groups of the fibre at least one  $\beta$ -(2,2,3,3-tetrafluorocyclobutyl)-acryloylamino or a vinylsulfone group or at least one group forming in an alkaline medium a vinyl-sulfone group by using in said process padding liquors containing in addition to the above-mentioned dyestuffs as agents having alkaline action a liquid alkali metal silicate.

This application is a continuation of application Ser. No. 706,766, filed Feb. 20, 1968, now abandoned.

It is known that textile materials made of cellulose fibres can be dyed with reactive dyestuffs having as component capable of reacting the  $\beta$ -(2,2,3,3-tetrafluorocyclobutyl)-acryloylamino- or vinylsulfone group or a group forming in the presence of alkalies a vinylsulfone group, by allowing to react these reactive dyestuffs under alkaline conditions with the hydroxyl groups of the cellulose fibres. As agents having alkaline action generally inorganic alkalies such, for example, as soda, sodium bicarbonate, trisodium phosphate, sodium hydroxide, sodium metasilicate ( $\text{Na}_2\text{SiO}_3 \cdot 5\text{H}_2\text{O}$ ) or mixtures of these alkalies are used. In the alkaline medium of the dyeing baths which are applied in this manner, during the dyeing process, not only the reaction of the fore-mentioned reactive groups with the hydroxyl groups of the cellulose fibres takes place but also, to a certain extent, a simultaneous reaction of said groups with the water from the bath occurs as secondary reaction. Caused by this secondary reaction, more or less large portions of the dyestuff used are lost for the actual dyeing. In this instance, the stronger the alkalies used, the higher the temperature of the bath and the longer the dwelling period of the dyestuffs in the alkaline dyebath, the lower the stability of such dyestuffs in the dyebath. With the usual processes for pad-dyeing it is known that the dwelling period plays an especially important role in the quality of the dyeings prepared. Within this method of working, the dyeing liquor which is kept in a storage container or a preparing vessel is led gradually into the padding machine. This measure, however, has negative effects when larger batches are dyed for which a large amount of a dyebath is necessary, so that occasionally a time difference of about more than one hour between the application of the first and the last liter of the dyeing bath arises, which is padded in the padding machine on the textile material. If, during this period, a noticeable reaction of the dyestuffs with the water takes place, the colour yield is continuously reduced so that, consequently, goods are obtained showing end-to-end tailing, i.e. the initial portion being a darker shade than the final portion. The danger of end-to-end tailing of the dyed goods is present even when the temperature of the padding liquor cannot be kept below 20-25°C., as is often the case in countries having a hot climate.

2

Therefore, metering pumps or mixing devices are brought into action in such padding processes in which, generally, relatively large amounts of strong alkalies (for example sodium hydroxide or sodium metasilicate) are used and in which—especially when large batches are dyed—the dyebath is abandoned partially for a prolonged period of time in the preparing vessel. Said arrangements allow the dissolved dyestuffs to be brought into contact with the alkali only shortly before they are introduced into the padding machine (cf. Textil-Praxis, 1963, page 1189). A disadvantage of this process, however, is that only few dye-houses possess such metering pumps or mixing devices, which is due to the high purchase price for such devices.

An important padding process for fixing the above-mentioned dyestuffs on fabrics made of cellulose fibres is in this respect the so-called "pad-batch-process" or a variation thereof, the so-called "pad-short-dwell-process" (cf. SVF-Fachorgan 1961, page 320, as well as Textil-Praxis 1963, page 1189). According to these processes the textile material is wound up on a roller and allowed to dwell, the wound up textile material being, during the dwelling time, hermetically enveloped in order to prevent the carbon dioxide from the air reacting with the alkalies at the edges of the rolled up material, which would then result in only an insufficient dyestuff fixation in these areas.

It is also possible in the above-mentioned processes, to work without a metering pump, but only weak alkalies such, for example, as soda or alkali metal bicarbonate are allowed then to be used. These substances, however, reduce the colour yield due to the insufficient fixation quote of the dyestuffs on the fibre. Furthermore, the application of weak alkalies in this process may run the risk that, particularly when dyeing greater batches, the edges of the initial portion of the padded, rolled-up material become lighter coloured on account of the long period during which the textile material is rolled up.

A further disadvantage of the pad-batch- or the pad-short-dwell-process lies in the fact that after dwelling, when drying the textile material without preceding acidification of the goods, the colour yield is reduced, owing to cleavage of the dyestuff-fibre-linkage. Therefore it is inappropriate to use the non after-treated textile material in the printing.

It has now been found that textile materials made of native or regenerated cellulose fibres can be dyed according to the padding process with reactive dyestuffs having as a group capable of reacting at least one  $\beta$ -(2,2,3,3-tetrafluorocyclobutyl)-acryloylamino group or a vinylsulfone group or at least one group forming in an alkaline medium a vinyl sulfone group, by using in said process padding liquors containing besides the above-mentioned dyestuffs as agents having alkaline action a liquid alkali metal silicate. For the fixation of the dyeings, the padded material is allowed to dwell at temperatures of up to 100°C., preferably at room temperature, the fabric being wound up on a roller or piled up. The dwelling period is generally between 1 hour and 30 hours.

By the addition of alkali metal silicate (water glass) when carrying out the process of the present invention a metering pump or a mixing device is no longer necessary for padding the textile material, without risking the formation of lighter coloured edges or the so-called end-to-end tailing of the treated material. Furthermore, this mode of operation according to the present process allows the drying of the dyeings before acidification of the goods.

The present invention may also be applied in the same manner and with the same advantages on mixed fabrics consisting of native and regenerated cellulose.

As reactive dyestuffs representatives of the various organic dyestuff classes can be used according to the present invention, for example azo- and anthraquinone dyestuffs, containing either at least one  $\beta$ -(2,2,3,3-tetrafluoro-cyclobutyl)-acryloylamino- or a vinylsulfone group or at least one group which can be converted into a vinylsulfone group when exposed to alkaline agents during the dyeing process. The appropriate azo dyestuffs may, if desired, be used in metallized form.

As examples for such groups in the dyestuffs to be applied which can be converted into the vinylsulfone group in the presence of substances having alkaline reaction during the dyeing process, there are mentioned in particular the sulfuric acid ester or thiosulfuric acid ester of  $\beta$ -hydroxyethylsulfone groupings.

Of the liquid alkali metal silicates (water-glasses) which are added to the padding baths according to the process of the present invention there are suitably used the commercial sodium silicates (soda water glass). Preferably there are used sodium silicates having a concentration of about 37° to about 60° Bé., corresponding to an  $\text{SiO}_2$ -content of the aqueous solution of about 27.2 to about 38.2 percent by weight.

The amount of the fixing agent used depends on the concentration of the alkali metal silicate applied, on the dyestuff concentration and on the nature of the dyestuff, and ranges generally from about 25 g. to about 350 g., preferably from about 50 g. to 200 g. per liter of padding bath. Furthermore, it is possible to add to the dye baths still a sodium hydroxide solution besides the silicate, but the amount of sodium hydroxide solution (referred to sodium hydroxide solution of 38° Bé.) is not to exceed 10% of the amount of alkali metal silicate used, since otherwise the stability of the bath is reduced.

The technical advantage which is achieved when using liquid alkali metal silicates as fixing agents lies in the fact that sources of error are avoided which are possible when preparing the conventional aqueous padding liquors, an excellent reproducibility of the desired tints is guaranteed, and the dyeings do not suffer a change of shade during the dwelling period. It is surprising that with the process of the present invention, besides an excellent colour yield and levelness of the dyeing, still an excellent tone-in-tone dyeing on mixed fabrics made of native or regenerated cellulose fibre is obtained which is superior to that according to known conventional processes when other alkalies are used such, for example, as sodium hydroxide solution, trisodium phosphate, soda, an alkali metal bicarbonate or metasilicate.

The following Examples serve to illustrate the invention but they are not intended to limit it thereto.

#### EXAMPLE 1

A cotton poplin is padded in a padding machine—without using a metering pump or mixing device—at a squeezing effect of 70 percent by weight with a padding liquor of 30° C. containing per liter of water 10 g. of the dyestuff of the formula



in commercial form and condition, and 200 g. of sodium silicate of 49° Bé. After padding the fabric is rolled up continuously and allowed to dwell at 30° C. for 24 hours. Then the dyed fabric is rinsed, acidified and soaped as usual.

There is obtained a brilliant red dyeing of excellent colour yield and having level coloured ends and edges.

#### EXAMPLE 2

5 A mercerized cotton fabric is padded in a padding machine—without using a metering pump or a mixing device—at a squeezing effect of 80 percent by weight with a padding liquor of 20° C. containing per liter of water 20 g. of the dyestuff of the formula



in commercial form and condition, and 200 g. of sodium silicate of 49° Bé. After padding the fabric is rolled up continuously and allowed to dwell at 20° C. for 6 hours. Then the dyed goods are rinsed, acidified and soaped.

15 There is obtained a brilliant orange dyeing of an excellent colour yield and having level coloured ends and edges.

#### EXAMPLE 3

20 A mercerized cotton fabric is padded in a padding machine—without using a metering pump or a mixing device—at a squeezing effect of 80 percent by weight with a padding liquor of 20° C. containing per liter of water 40 g. of the dyestuff of the formula



35 in commercial form and condition, and 50 g. of sodium silicate of 49° Bé. After padding the fabric is rolled up continuously and allowed to dwell at 20° C. for 24 hours. Then the dyed goods are rinsed as usual, acidified and soaped.

40 There is obtained a brilliant violet dyeing of an excellent colour yield and having level coloured ends and edges.

#### EXAMPLE 4

45 A mercerized cotton fabric is padded in a padding machine—without using a metering pump or a mixing device—at a squeezing effect of 80 percent by weight with a padding liquor of 30° C. containing per liter of water 20 g. of the dyestuff of the formula



60 in commercial form and condition, and 300 g. of sodium silicate of 49° Bé. After padding the fabric is rolled up continuously and allowed to dwell at 30° C. for 6 hours. Then the dyed goods are rinsed as usual, acidified and soaped.

65 There is obtained a brilliant yellow dyeing of an excellent colour yield and having level coloured ends and edges.

#### Example 5

70 A mercerized cotton fabric is padded in a padding machine—without using a metering pump or a mixing device—at a squeezing effect of 80 percent by weight with a

padding liquor of 30° C. containing per liter of water 30 g. of the dyestuff of the formula



in commercial form and condition, and 200 g. of sodium silicate of 49° Bé. After padding the fabric is rolled up continuously and allowed to dwell at 30° C. for 4 hours. Then the dyed goods are rinsed as usual, acidified and soaped.

There is obtained a brilliant blue dyeing of an excellent colour yield and having level coloured ends and edges.

If, in the Example described above, after dwelling, the fabric is dried for 3 minutes at 140° C. and then rinsed, acidified and soaped, as usual, a level dark blue dyeing is obtained likewise; re-cleavage of the dyestuff-fibre-linkage, caused while drying, could not be ascertained from the colouristic aspect.

#### Example 6

A fabric made of staple fibre is padded in a padding machine—without using a metering pump or a mixing device—at a squeezing effect of 90 percent by weight with a padding liquor of 20° C. containing per liter of water 40 g. of the dyestuff of the formula



in commercial form and composition, and 200 g. of sodium silicate of 49° Bé. After padding the fabric is rolled up continuously and allowed to dwell at 20° C. for 8 hours. Then the dyed goods are rinsed as usual, acidified and soaped.

There is obtained a brilliant red dyeing of an excellent colour yield and having level coloured ends and edges.

#### Example 7

A cotton fabric is padded in a padding machine—without using a metering pump or a mixing device—at a squeezing effect of 80 percent by weight with a padding liquor of 20° C. containing per liter of water 70 g. of the dyestuff of the following formula



in commercial form and composition, and 150 g. of sodium silicate of 49° Bé. After padding the fabric is rolled up continuously and allowed to dwell at 20° C. for 18 hours. Then the dyed goods are rinsed, acidified and soaped, as usual.

There is obtained a blue dyeing of an excellent colour yield and having level coloured ends and edges.

#### Example 8

A mixed fabric of staple fibre and cotton in a mixing proportion of 30:70 is padded in a padding machine—without using a metering pump or a mixing device—at a squeezing effect of 80 percent by weight with a padding

liquor of 30° C. containing per liter of water 20 g. of the dyestuff of the formula



in commercial form and composition, and 200 g. of sodium silicate of 49° Bé. After padding the mixed fabric is rolled up continuously and allowed to dwell at 30° C. for 8 hours. Then the dyed goods are rinsed as usual, acidified and soaped.

There is obtained a yellow tone-in-tone dyeing of an excellent colour yield having level coloured ends and edges.

#### Example 9

A staple fibre fabric is padded in a padding machine at a squeezing effect of 90 percent by weight with a padding liquor of 40° C. containing per liter of water 20 g. of the dyestuff of the formula



in commercial form and composition, 50 g. of sodium silicate of 49° Bé and 5 cc. of a sodium hydroxide solution of 38° Bé. After padding the fabric is rolled up continuously and allowed to dwell at 40° C. for 24 hours. Then the dyed goods are rinsed, acidified and soaped, as usual.

There is obtained a brilliant orange dyeing having level coloured ends and edges.

#### Example 10

A mercerized cotton fabric is padded in a padding machine at a squeezing effect of 60 percent by weight with a padding liquor of 30° C. containing per liter of water 20 g. of the dyestuff of the formula



in commercial form and composition, 150 g. of sodium silicate of 49° Bé. and 7.5 cc. of a sodium hydroxide solution of 38° Bé. After padding the fabric is rolled up continuously and allowed to dwell at 30° C. for 12 hours.

There is obtained an orange dyeing having level coloured end and edges.

#### Example 11

A bleached linen fabric is padded in a padding machine at a squeezing effect of 80 percent by weight with a padding liquor of 20° C. containing per liter of water 15 g. of the dyestuff of the formula



in commercial form and composition, and 200 g. of sodium silicate of 49° Bé. After padding the fabric is rolled up continuously and allowed to dwell at 20° C. for 24 hours.

There is obtained a red dyeing having level coloured ends and edges.

Example 12

A mercerized cotton fabric is padded in a padding machine at a squeezing effect of 60 percent by weight with a padding liquor of 20° C. containing per liter of water 10 20 g. of the dyestuff of the formula



in commercial form and composition, and 200 g. of sodium silicate of 49° Bé. After padding the fabric is rolled up continuously and allowed to dwell at 20° C. for 24 20 hours.

There is obtained a yellow dyeing having level coloured ends and edges.

Example 13

A mercerized cotton fabric is padded in a padding machine at a squeezing effect of 60 percent by weight with a padding liquor of 20° C. containing per liter of water 30 g. of the dyestuff of the formula



in commercial form and composition, and 50 g. of sodium silicate of 49° Bé. After padding the fabric is rolled up continuously and allowed to dwell for 24 hours.

There is obtained a yellow dyeing having level coloured 45 ends and edges.

I claim:

1. In a process for pad-dyeing textile materials made of or containing native or regenerated cellulose fibers with dyestuffs having as group capable of reacting with the hydroxyl groups of the fiber at least one  $\beta$ -(2,2,3,3-tetrafluoro-cyclobutyl)-acryloylamino or vinylsulfone group or sulfatoethylsulfone or thiosulfatoethylsulfone group, and fixing the dyestuffs according to the dwelling method, the improvement which comprises: using in said process, padding liquors containing, in addition to the said dyestuffs, as an agent having alkaline reaction, a liquid sodium silicate having a concentration in the range of from 37° to 60° Bé., corresponding to an SiO<sub>2</sub>-content of the aqueous solution of 27.2 to 38.2 percent by weight, in an amount ranging from 25 grams to 350 grams per liter of padding liquor.

2. A process as claimed in Claim 1, wherein the liquid sodium silicate is used in an amount of from 50 grams to 200 grams per liter of padding liquor.

3. A process as claimed in Claim 1, wherein padding liquors are used which additionally contain a sodium hydroxide solution, the amount thereof, calculated as sodium hydroxide solution of 38° Bé., not exceeding ten percent by weight of the amount of sodium silicate used.

4. A process as claimed in Claim 1, wherein for the fixation of the dyeings, the textile material padded with reactive dyestuff and sodium silicate is batched up on a roller and is allowed to dwell there at temperatures ranging from room temperature up to 100° C.

5. A process as claimed in Claim 1, wherein for the fixation of the dyeings, the textile material padded with reactive dyestuff and sodium silicate is cutted up and is allowed to dwell there at temperatures ranging from room temperature up to 100° C.

References Cited

UNITED STATES PATENTS

|           |         |                      |         |
|-----------|---------|----------------------|---------|
| 3,232,927 | 2/1966  | Randall et al. ----- | 260—163 |
| 3,129,052 | 4/1964  | Dawson et al. -----  | 8—54    |
| 3,360,505 | 12/1967 | Scherer et al. ----- | 260—147 |

ROLAND E. MARTIN, JR., Primary Examiner

U.S. CL. X.R.

8—1 P, 1 Q, 39, 41 R, 42 R, 82